# EUROPEAN PATENT SPECIFICATION

(11) **EP 3 126 537 B1**
(45) Date of publication and mention of the grant of the patent: **13.05.2020**
(21) Application number: 15712762.2
(22) Date of filing: 12.03.2015
(51) Int. Cl.: C22C 38/40, C22C 38/42, C22C 38/44, C22C 38/02, C22C 38/04, C22C 38/54, C22C 38/00, C21D 6/00, C21D 8/02

(54) **DUAL-PHASE STAINLESS STEEL**
ZWEIPHASIGER EDELSTAHL
ACIER INOXYDABLE À DEUX PHASES

(30) Priority: 01.04.2014 US 201414231778
(43) Date of publication of application: 08.02.2017
(73) Proprietor: ATI Properties LLC, Albany OR 97321 (US)
(72) Inventor: BERRY, David C., Washington, PA 15301 (US); BAILEY, Ronald E., Pittsburgh, PA 15216 (US)
(74) Representative: Potter Clarkson
(86) International application number: PCT/US2015/020122
(87) International publication number: WO 2015/153092

(56) References cited:
- EP-A1- 1 876 253
- EP-A1- 2 172 573
- CN-A- 102 899 587
- JP-A- S5 453 615
- JP-A- 2000 008 144
- JP-A- 2008 138 270
- KR-A- 20030 037 751
- US-A- 4 608 099
- US-A1- 2008 069 719

## Description

### FIELD OF TECHNOLOGY

The present disclosure relates to a dual-phase stainless steel having a microstructure of ferrite and tempered martensite. In particular, the present disclosure relates to cost-effective stainless steels having improved hardness for abrasion-resistant and/or wear-resistant applications.

### DESCRIPTION OF THE BACKGROUND OF THE TECHNOLOGY

Dual-phase stainless steels can exhibit a combination of desirable properties that make them useful for a wide variety of industrial applications, such as for oil sands extraction and in the sugar industry. These steels are generally characterized by a microstructure of tempered martensite dispersed in a ferrite matrix.

An example of a dual-phase stainless steel is ATI 412™ stainless steel (UNS 41003), which typically contains, by weight, 11.75% chromium (Cr), 0.90% manganese (Mn), 0.70% silicon (Si), 0.40% nickel (Ni), 0.030% sulfur (S), 0.020% carbon (C), 0% to 0.040% phosphorus (P), 0% to 0.030% nitrogen (N), and the balance iron (Fe) and other incidental impurities. ATI 412™ stainless steel typically has a Brinell hardness (HB) of about 177 when annealed at about 766° C., and a Brinell hardness of about 258 when annealed at about 843° C.

Another dual-phase stainless steel is Duracorr® steel, which contains, by weight, 11.0% to 12.5% Cr, 0.20% to 0.35% molybdenum (Mo), 0% to 1.50% Mn, 0% to 1.00% Ni, 0% to 0.70% Si, 0% to 0.040% P, 0% to 0.030% N, 0% to 0.025% C, 0% to 0.015% S, and the balance Fe. Notably, Duracorr® stainless steel contains Mo as an alloying element, i.e., an intentional alloying addition, and not as an incidental impurity. Because of the rising costs of Mo, however, Duracorr® stainless steel may be too costly for certain applications. Although Duracorr® stainless steel typically has a hardness of about 223 HB, it can be processed to exhibit nominal hardness of 300 HB, which grade is commercially available as Duracorr® 300 stainless steel. Duracorr® and Duracorr® 300 stainless steels have largely the same composition, but the hardness of Duracorr® 300 stainless steel varies from 260 HB to 360 HB. The increased hardness of Duracorr® 300 stainless steel, however, is accompanied by a reduction in toughness. For example, the Charpy V-notch impact energy of Duracorr® 300 stainless steel at -40° C. is only about 20.3 N-m (15 ft-lb) on average.
KR20030037751A discloses a method of manufacturing 12Cr ferritic and martensitic hot rolled stainless steel. The method includes the steps of hot rolling a steel slab comprising 0.03 wt.% or less of C, Cr 11 to 13.5 wt.%, 1.0 wt.% or less of Ni, 1.0 wt.% or less of Si, 0.2 wt.% or less of Mo, 1.0 wt.% or less of Cu, 1.0 wt.% or less of Mn, a balance of Fe and incidental impurities; heat treating the hot rolled steel sheet in a specified temperature range for at least 10 min, followed by cooling.

CN102899587A relates to a double phase stainless steel, which comprises the following chemical components, by weight: less than or equal to 0.02% of C, less than or equal to 0.02% of N, less than or equal to 0.03% of P, less than or equal to 0.015% of S, less than or equal to 0.35% of Si, 1.0-3.0% of Mn, 10.5-13.5% of Cr, 0.5-1.5% of Ni, 8(C+N)-0.35% of Ti, 0.10-0.30% of Nb+Mo, and the balance of Fe and unavoidable impurities, wherein the ferrite factor KFF is in 6.0-11.5.

JP2008138270A relates to a high strength Cr-containing stainless steel sheet having excellent workability. The high strength stainless steel sheet having excellent workability has a composition comprising, by mass, 0.001 to 0.03% C, 0.001 to 0.03% N, 0.05 to 0.5% Si, 0.05 to 5% Mn, ≤0.05% P, 0.3 to 5% Ni, 0.01 to 3% Cu, 10 to 18% Cr and 0.005 to 0.50% Al, and the balance Fe with inevitable impurities.

In applications requiring a stainless steel having abrasion resistance and/or wear resistance, high hardness levels, for example, up to about 350 HB, may be desirable in combination with higher toughness than is available from Duracorr® 300 stainless steel. Moreover, an in-service work hardenability up to about 450-500 HB, for example, may be required in certain applications. Furthermore, it is desirable that any such alloys are cost-effective

### SUMMARY

The invention provides a dual-phase ferritic-martensitic stainless steel in accordance with claim 1 of the appended claims.
According to one non-limiting aspect of the present disclosure, an embodiment of a high-hardness dual-phase ferritic-martensitic stainless steel is described. The stainless steel comprises, by weight, 11.5% to 12% Cr, 0.8% to 1.5% Mn, 0.75% to 1.5% Ni, 0% to 0.5% Si, 0% to 0.2% Mo, up to 0.0025% B, Fe, and impurities. The stainless steel according to the present disclosure exhibits Brinell hardness (HB) of 300 HB or greater and Charpy V-notch impact energy at -40°C (CVN) such that CVN (ft-lb)+(0.4×HB) is 160 or greater.

According to another non-limiting aspect of the present disclosure, an embodiment of an article of manufacture including a high-hardness dual-phase ferritic-martensitic stainless steel is described. The stainless steel comprises, by weight, 11.5% to 12% Cr, 0.8% to 1.5% Mn, 0.75% to 1.5% Ni, 0% to 0.5% Si, 0% to 0.2% Mo, up to 0.0025% B, Fe, and impurities. The stainless steel exhibits Brinell hardness (HB) of 300 HB or greater and Charpy V-notch impact energy at -40°C (CVN) such that CVN (ft-lb)+(0.4xHB) is 160 or greater.

### BRIEF DESCRIPTION OF THE DRAWING

Features and advantages of the stainless steels and articles of manufacture described herein may be better understood by reference to the accompanying drawing in which:
Figure 1 is a graph plotting Brinell hardness and Charpy V-notch impact energy of non-limiting embodiments of stainless steels according to the present disclosure in comparison to certain conventional steels.

The reader will appreciate the foregoing details, as well as others, upon considering the following detailed description of certain non-limiting embodiments of stainless steels and articles of manufacture according to the present disclosure. The reader also may comprehend certain of such additional details upon making or using the stainless steels and articles of manufacture described herein.

### DETAILED DESCRIPTION OF CERTAIN NON-LIMITING EMBODIMENTS

The invention is defined in the claims.

The present disclosure, in part, is directed to cost-effective dual-phase ferritic-martensitic stainless steels having advantageous hardness and which are suitable for use in various applications requiring abrasion resistance and/or wear resistance. In particular, embodiments of dual-phase ferritic-martensitic stainless steels according to the present disclosure comprise, by weight, 11.5% to 12% Cr, 0.8% to 1.5% Mn, 0.75% to 1.5% Ni, 0% to 0.5% Si, 0% to 0.2% Mo, up to 0.0025% B, Fe, and impurities. The stainless steels exhibit Brinell hardness (HB) of 300 HB or greater and Charpy V-notch impact energy at -40°C (CVN) such that the following is satisfied: CVN (ft-lb)+(0.4×HB) is 160 or greater.

Cr may be provided in the alloys of the present disclosure to impart corrosion resistance. A Cr content of about 11.5% (by weight) or more may be required to provide adequate corrosion resistance. On the other hand, excessive Cr may undesirably (1) stabilize the ferrite phase and/or (2) embrittling phases such as the sigma phase. Accordingly, embodiments of the stainless steels according to the present disclosure include a Cr content of 11.5% to 12%, by weight.

Mn may be provided in the alloys of the present disclosure to improve work hardenability. A Mn content of about 0.8% (by weight) or more may be required to achieve the desired work hardening effects. On the other hand, excessive Mn may undesirably segregate during processing of the stainless steels. Accordingly, embodiments of the stainless steels according to the present disclosure include a Mn content of 0.8% to 1.5%, by weight. In certain other embodiments, the Mn content of the stainless steels may be 1.0% to 1.5%, by weight. In certain embodiments of the stainless steels according to the present disclosure, the addition of Mn in combination with the addition of other alloying elements can advantageously affect work hardenability such that the steels attain a hardness of 450 HB or greater.

Ni may be provided in the alloys of the present disclosure to help stabilize the martensitic phase of the dual-phase (martensitic-ferritic) alloys. A Ni content of about 0.75% by weight or more may be required to provide a material including higher levels of martensite than in Duracorr® 300 stainless steel. Without intending to be bound to any theory, the nickel content of the alloys may promote hardness of the alloys' martensite phase by stabilizing austenite formation during heat treatment, allowing more time for carbon diffusion. On the other hand, due to the high cost of Ni, it may be desirable to limit the Ni content. Accordingly, embodiments of the steels according to the present disclosure include a Ni content of 0.75% to 1.5% (by weight) to provide a cost-effective dual-phase stainless steel with high hardness levels up to about 350 HB, in combination with higher toughness than is typical of Duracorr® 300 stainless steel. In further embodiments, the Ni content of stainless steels according to the present disclosure may be 1.0% to 1.5%, by weight.

In certain embodiments of the stainless steels according to the present disclosure, the level of Si may be limited to (1) destabilize the ferritic phase of the dual-phase stainless steels and/or (2) avoid embrittling phases such as the sigma phase. Accordingly, certain embodiments of the steels according to the present disclosure include 0% to no more than about 0.5% Si, by weight.

In certain embodiments of the stainless steels according to the present disclosure, the level of Mo may be limited to (1) destabilize the ferritic phase of the dual-phase stainless steels and/or (2) avoid embrittling phases such as the sigma phase. Accordingly, embodiments of the steels according to the present disclosure include 0% to no more than 0.2% Mo, by weight. In certain other embodiments of the steels according to the present disclosure, the Mo concentration is 0% to no more than 0.1%, by weight.

B may be provided in the dual-phase stainless steels of the present disclosure to improve martensite hardness. Steels of the present disclosure may include up to 0.0025% B, by weight. In certain embodiments of the steels, the B content is 0.002% to 0.0025%, by weight.

Incidental elements and impurities in the disclosed alloys may include, for example, one or more of C, N, P, and S. In certain embodiment of the stainless steels according to the present disclosure, the total content of these elements is no more than 0.1%, by weight. In certain embodiments, C may be present in the steels disclosed herein in an amount no more than 0.025%, by weight. In certain embodiments, S may be present in the steels disclosed herein in an amount no more than 0.01%, by weight. In certain embodiments, N may be present in the steels disclosed herein in an amount no more than 0.03%, by weight. Incidental levels of various metallic elements also may be present in embodiments of alloys according to the present disclosure. For example, certain non-limiting embodiments of alloys according to the present disclosure may include up to 0.25% copper (Cu), by weight.

According to certain non-limiting embodiments, dual-phase ferritic-martensitic stainless steels according to the present disclosure comprise by weight: 11.5% to 12% Cr; 1.0% to 1.5% Mn; 1.0% to 1.5% Ni; 0% to 0.5% Si; 0% to 0.1% Mo; up to 0.0025% B; 0% to 0.025% C; 0% to 0.01% S; 0% to 0.03% N, Fe, and impurities. In certain embodiments, the stainless steels further comprise P. In certain embodiments, the total concentration of C, N, P, and S is no greater than 0.1%, by weight. In certain embodiments the concentration of B in the steels is 0.002% to 0.0025%, by weight. The steels include no more than 0.25% Cu, by weight.

According to certain non-limiting embodiments, dual-phase ferritic-martensitic stainless steels according to the present disclosure consist essentially of, by weight: 11.5% to 12% chromium; 0.8% to 1.5% manganese; 0.75% to 1.5% nickel; 0% to 0.5% silicon; 0% to 0.2% molybdenum; up to 0.0025% boron; 0% to 0.025% carbon; 0% to 0.01% sulfur; 0% to 0.03% nitrogen; optionally at least one of copper and phosphorus; iron; and impurities.

According to certain non-limiting embodiments, dual-phase ferritic-martensitic stainless steels according to the present disclosure consist essentially of, by weight: 11.5% to 12% chromium; 1.0% to 1.5% manganese; 1.0% to 1.5% nickel; 0% to 0.5% silicon; 0% to 0.1% molybdenum; up to 0.0025% boron; 0% to 0.025% carbon; 0% to 0.01% sulfur; 0% to 0.03% nitrogen; optionally at least one of copper and phosphorus; iron; and impurities.

According to certain non-limiting embodiments, dual-phase ferritic-martensitic stainless steels according to the present disclosure consist of, by weight: 11.5% to 12% chromium; 0.8% to 1.5% manganese; 0.75% to 1.5% nickel; 0% to 0.5% silicon; 0% to 0.2% molybdenum; up to 0.0025% boron; 0% to 0.025% carbon; 0% to 0.01% sulfur; 0% to 0.03% nitrogen; optionally at least one of copper and phosphorus; iron; and impurities.

According to certain non-limiting embodiments, dual-phase ferritic-martensitic stainless steels according to the present disclosure consist of, by weight: 11.5% to 12% chromium; 1.0% to 1.5% manganese; 1.0% to 1.5% nickel; 0% to 0.5% silicon; 0% to 0.1% molybdenum; up to 0.0025% boron; 0% to 0.025% carbon; 0% to 0.01% sulfur; 0% to 0.03% nitrogen; optionally at least one of copper and phosphorus; iron; and impurities.

For a given steel, hardness is generally inversely related to toughness. In the present disclosure, Brinell hardness (HB) is the primary measure of hardness, and Charpy V-notch impact energy at -40°C (CVN) is the primary measure of toughness. Referring to Fig. 1, for certain embodiments of the steels according to the present disclosure, CVN (ft-lb)+(0.4xHB) of the steels is about 160 or greater. In certain embodiments of the steels according to the present disclosure, hardness is about 300 HB or greater, and CVN is about 67.8 N-m (50 ft-lb) or greater. In certain embodiments, the steels according to the present disclosure have an in-service work hardenability up to a hardness of about 450 HB or greater.

### EXAMPLES

Table 1 includes the compositions and certain properties of an embodiment of the dual-phase ferritic-martensitic stainless steels according to the present disclosure and of conventional ATI 412™ stainless steel and conventional Duracorr® 300 stainless steel. Heats of the three alloys listed in Table 1 were melted into slabs weighing about 6818 kg (15,000 lb) and rolled at a temperature of about 1066°C (1950°F) to produce material about 6 mm thick. Following the rolling process, the steels were annealed at 766°C or 843°C, for 15 minutes, and air cooled.

The mechanical properties of the experimental steel embodiment listed in Table 1 were measured and compared to those of the two listed conventional steels. The Brinell hardness and CVN at -40°C (ft-lb) are shown in Table 1 for the three alloys. The tensile tests were conducted according to the American Society for Testing and Materials (ASTM) standard A370 at room temperature, using a tungsten carbide ball indenter, on samples measuring about 5 cm in gauge length and about 0.5 cm in thickness. The Charpy tests were conducted according to ASTM standard A370 and E23 at about -40°C on transverse samples measuring about 10 mm × 2.5 mm. Because these samples are considered subsize per ASTM-A370, the measured impact energy was converted to standard size specimen values in Table 1.

As shown by the experimental results in Table 1, the experimental steel sample of the present disclosure exhibited very favorable hardness and toughness (CVN impact energy) relative to the conventional alloys. This was particularly unexpected and surprising. Commercially available alloys providing comparable hardness and toughness typically are carbon steels, which would not withstand corrosive environments.

In certain possible non-limiting embodiments, dual-phase stainless steels according to the present disclosure are prepared using conventional stainless steel production practices including, for example, melting of starting materials in an electric furnace, decarburization via AOD, and casting to an ingot. Ingots may be cast, for example, by continuous casting or ingot pouring. In certain embodiments, the cast material may be heat treated (austenitized) or sold as-rolled.

**Table 1**

| | Embodiment of Present Steel | | Conventional Steels | | |
|---|---|---|---|---|---|
| wt% | | | ATI 412™ Alloy | | Duracorr® Alloy |
| C | 0.022 | | 0.01-0.025 | | 0-0.025 |
| Mn | 0.89 | | 0.8-1 | | 0-1.5 |
| P | 0.027 | | 0-0.04 | | 0-0.04 |
| S | 0.0014 | | 0-0.004 | | 0-0.015 |
| Si | 0.44 | | 0.45-0.75 | | 0-0.7 |
| Cr | 11.92 | | 11.5-12 | | 11-12.5 |
| Ni | 0.97 | | 0.3-0.75 | | 0-1 |
| N | 0.023 | | 0-0.03 | | 0-0.03 |
| Mo | 0.091 | | 0-0.2 | | 0.2-0.35 |
| Cu | 0.17 | | 0.25 | | 0 |
| B | 0.0003 | | 0 | | 0 |
| Annealing temperature | As-rolled | 843°C | 766°C | 843°C | - |
| Brinell hardness | 340 | 322 | 177 | 258 | 260-360 |
| CVN at -40°C (ft-lb) | 26-34 | 56-62 | 65-90 | 7-49 | 15 |
| CVN)ft-lb)+(0.4xHB) | 162-170 | 185-191 | 136-161 | 111-152 | 119-159 |

The potential uses of alloys according to the present disclosure are numerous. As described and evidenced above, the dual-phase stainless steels described herein are capable of being used in many applications where abrasion resistance and/or wear resistance is important. Articles of manufacture for which the steels according to the present disclosure would be particularly advantageous include, for example, parts and equipment used in oil sands extraction and parts and equipment used in sugar processing. Other applications for the stainless steels according to the present disclosure will be readily apparent to ordinarily skill practitioners. Those having ordinary skill may readily manufacture these and other articles of manufacture from the stainless steels according to the present disclosure using conventional manufacturing techniques.

Although the foregoing description has necessarily presented only a limited number of embodiments, those of ordinary skill in the relevant art will appreciate that various changes in the alloys and article and other details of the examples that have been described and illustrated herein may be made by those skilled in the art, and all such modifications will remain within the principle and scope of the present disclosure as expressed herein and in the appended claims.

## Claims

1. A dual-phase ferritic-martensitic stainless steel consisting of, by weight:
11.5% to 12% chromium;
0.8% to 1.5% manganese;
0.75% to 1.5% nickel;
≤ 0.5% silicon;
≤ 0.2% molybdenum;
≤ 0.0025% boron;
≤ 0.25% copper;
≤ 0.025% carbon;
≤ 0.01% sulfur;
≤ 0.03% nitrogen;
wherein the total concentration of carbon + nitrogen + sulfur + phosphorus ≤ 0.1 %; balance iron and incidental impurities;
wherein the steel has a Brinell hardness (HB) of 300 HB or greater and a Charpy V-notch impact energy at -40°C (CVN) such that CVN (ft-lb) + (0.4 x HB) is about 160 or greater.

2. The dual-phase ferritic-martensitic stainless steel of claim 1, wherein boron content is 0.002% to 0.0025%.

3. The dual-phase ferritic-martensitic stainless steel of claim 1 or claim 2, wherein molybdenum content is ≤ 0.1 %.

4. The dual-phase ferritic-martensitic stainless steel of any one of the preceding claims, wherein nickel content is 1.0% to 1.5%.

5. The dual-phase ferritic-martensitic stainless steel of any one of the preceding claims, wherein manganese content is 1.0% to 1.5%.

6. The dual-phase ferritic-martensitic stainless steel of any one of the preceding claims, wherein CVN of the steel is 67.8 N-m (50 ft-lb) or greater.

7. The dual-phase ferritic-martensitic stainless steel of any one of the preceding claims, wherein the steel has work hardenability up to a hardness of 450 HB or greater.

8. An article of manufacture including a dual-phase stainless steel as recited in any one of the preceding claims.

9. The article of manufacture of claim 8, wherein the article of manufacture is selected from parts and equipment used in oil sands extraction and parts and equipment used in sugar processing.

## Patentansprüche

1. Zweiphasiger ferritisch-martensitischer rostfreier Stahl, bestehend aus, nach Gewicht:
11,5 % bis 12 % Chrom;
0,8 % bis 1,5 % Mangan;
0,75 % bis 1,5 % Nickel;
≤ 0,5 % Silicium;
≤ 0,2 % Molybdän;
≤ 0,0025 % Bor;
≤ 0,25 % Kupfer;
≤ 0,025 % Kohlenstoff;
≤ 0,01 % Schwefel;
≤ 0,03 % Stickstoff;
wobei die Gesamtkonzentration von Kohlenstoff + Stickstoff + Schwefel + Phosphor ≤ 0,1 %;
Reste an Eisen und zufällige Verunreinigungen;
wobei der Stahl eine Brinellhärte (HB) von 300 HB oder mehr und eine Charpy-Kerbschlagbiegeenergie bei -40 °C (*Charpy-V-notch* - CVN) derart aufweist, dass CVN (ft-lb) + (0,4 x HB) etwa 160 oder mehr beträgt.

2. Zweiphasiger ferritisch-martensitischer rostfreier Stahl nach Anspruch 1, wobei der Borgehalt 0,002 % bis 0,0025 % beträgt.

3. Zweiphasiger ferritisch-martensitischer rostfreier Stahl nach Anspruch 1 oder 2, wobei das Molybdängehalt ≤ 0,1 % beträgt.

4. Zweiphasiger ferritisch-martensitischer rostfreier Stahl nach einem der vorhergehenden Ansprüche, wobei der Nickelgehalt 1,0 % bis 1,5 % beträgt.

5. Zweiphasiger ferritisch-martensitischer rostfreier Stahl nach einem der vorhergehenden Ansprüche, wobei der Mangangehalt 1,0 % bis 1,5 % beträgt.

6. Zweiphasiger ferritisch-martensitischer rostfreier Stahl nach einem der vorhergehenden Ansprüche, wobei CVN des Stahls 67,8 Nm (50 ft-lb) oder mehr beträgt.

7. Zweiphasiger ferritisch-martensitischer rostfreier Stahl nach einem der vorhergehenden Ansprüche, wobei der Stahl eine Kaltumformung von bis zu einer Härte von 450 HB oder mehr aufweist.

8. Herstellungserzeugnis, das einen zweiphasigen rostfreien Stahl nach einem der vorhergehenden Ansprüche beinhaltet.

9. Herstellungserzeugnis nach Anspruch 8, wobei das Herstellungserzeugnis aus Teilen und Ausrüstungen, die bei der Ölsandextraktion verwendet werden, und Teilen und Ausrüstungen ausgewählt ist, die bei der Zuckerverarbeitung verwendet werden.

## Revendications

1. Acier inoxydable ferritique-martensitique biphasé constitué, en poids :
de 11, 5 % à 12 % de chrome ;
de 0,8 % à 1,5 % de manganèse ;
de 0,75 % à 1,5 % de nickel ;
≤ 0,5 % de silicium ;
≤ 0,2 % de molybdène ;
≤ 0,0025 % de bore ;
≤ 0,25 % de cuivre ;
≤ 0,025 % de carbone ;
≤ 0,01 % de soufre ;
≤ 0,03 % d'azote ;
dans lequel la concentration totale de carbone + azote + soufre + phosphore ≤ 0,1 % ;
le reste étant du fer et des impuretés accidentelles ;
l'acier ayant une dureté Brinell (HB) de 300 HB ou plus et une énergie d'impact de résilience Charpy V à -40 °C (CVN) telle que CVN (pi-lb) + (0,4 x HB) étant d'environ 160 ou plus.

2. Acier inoxydable ferritique-martensitique biphasé selon la revendication 1, dans lequel la teneur en bore est de 0,002 % à 0,0025 %.

3. Acier inoxydable ferritique-martensitique biphasé selon la revendication 1 ou la revendication 2, dans lequel la teneur en molybdène est ≤ 0,1 %.

4. Acier inoxydable ferritique-martensitique biphasé selon l'une quelconque des revendications précédentes, dans lequel la teneur en nickel est de 1,0 % à 1,5 %.

5. Acier inoxydable ferritique-martensitique biphasé selon l'une quelconque des revendications précédentes, dans lequel la teneur en manganèse est de 1,0 % à 1,5 %.

6. Acier inoxydable ferritique-martensitique biphasé selon l'une quelconque des revendications précédentes, dans lequel la CVN de l'acier est de 67,8 N m (50 pi-lb) ou plus.

7. Acier inoxydable ferritique-martensitique biphasé selon l'une quelconque des revendications précédentes, dans lequel l'acier est sensible à l'écrouissage jusqu'à une dureté de 450 HB ou plus.

8. Article manufacturé comportant un acier inoxydable biphasé selon l'une quelconque des revendications précédentes.

9. Article manufacturé selon la revendication 8, dans lequel l'article manufacturé est choisi parmi des pièces et équipements utilisés dans l'extraction des sables bitumineux et des pièces et équipements utilisés dans la transformation du sucre.
